

# UNITED STATES PATENT OFFICE.

ROBERT ABBOTT HADFIELD, OF SHEFFIELD, ENGLAND.

## HIGH-MANGANESE STEEL WITH LOW CARBON.

No. 856,250.

Specification of Letters Patent.

Patented June 11, 1907.

Application filed April 16, 1907. Serial No. 368,533.

*To all whom it may concern:*

Be it known that I, ROBERT ABBOTT HADFIELD, a subject of the King of Great Britain, and a resident of Sheffield, county of 5 York, England, have invented an Improvement in High-Manganese Steel with Low Carbon, of which the following description, in connection with the accompanying drawing, is a specification, like letters on the drawing representing like parts.

In the manufacture of high manganese steel, wherein the product is required to contain, say, from 10% to 14% and upward of manganese it has not heretofore been found practicable, or indeed commercially possible, 15 to keep the percentage of carbon as low as is desirable.

As a consequence of the comparatively and undesirably high percentage of carbon (owing 20 to the common use of ordinary ferro-manganese, containing from 6% to 9% of carbon) and because of the fact that manganese steel is a bad conductor of heat, it results that great care has to be taken in treating castings 25 and forgings made from such high manganese steel in order to avoid cracks therein or fracture thereof when they are being cooled, or when they are being heated preparatory to being subjected to a water toughening process, 30 as well as during such process and thereafter. In the course of my studies and experiments to overcome such objectionable features due to the high percentage of carbon in such steel I have discovered that by using, 35 in the manufacture of steel of the character specified, an alloy of manganese and iron low in carbon, that is, containing say less than 2% to 3% of carbon, instead of the ordinary ferro-manganese, I am enabled to produce a 40 magnetic high manganese steel in forms which have not heretofore been possible. This result is due to the fact that owing to the comparatively low percentage of carbon in the manganese steel made in accordance with 45 my invention the steel is rendered much less liable to fracture during the cooling, or heating and cooling treatment for toughening it hereinbefore mentioned, and such steel is distinguished by its relatively strong magnetic 50 character.

A low carbon manganese-iron alloy suitable for use in the manufacture of high manganese steel in accordance with my present invention is that now produced in the electric 55 furnace and which contains usually from 70% to 90% (seventy to ninety percent) of man-

ganese with less than 2% to 3% (two to three percent) of carbon.

In carrying out my invention low carbon manganese-iron alloy such as specified is 60 added, preferably in a molten condition, to a base of molten decarbonized iron, such as that used in the production of acid steel, and from which practically the whole of the carbon, silicon, and manganese have been eliminated in suitable manner, as for instance by the pneumatic or the open hearth method. The manganese alloy and the iron are preferably weighed in molten condition to insure that the resulting manganese steel shall accurately contain the desired percentage of manganese. The manganese steel thus produced is then poured into molds to form castings, or into molds to form ingots which are forged in any suitable manner requisite for 75 dealing with manganese steel.

By the process described I am enabled to produce in a practical manner and on a commercial scale a manganese steel having a much lower percentage of carbon than heretofore, and which steel can therefore be easily and readily heated and cooled with much less liability to fracture than heretofore.

A further advantage resulting from my invention is that articles can be safely made of 85 much thicker section of the improved manganese steel than of ordinary manganese steel. Thus, owing to the difficulties hereinbefore mentioned, and to the fact that higher percentage of carbon in manganese steel as 90 heretofore made tends to prevent as perfect or complete a toughening as is desirable, it has not heretofore been possible to produce on a practical scale, from high manganese steel, articles of more than about three or 95 four inches in thickness when the same required toughening. On the other hand articles can be made of the improved steel herein described of much thicker section while admitting of their being properly toughened. The steel made in accordance with my present invention is characterized by its relatively 100 strong magnetic quality.

The toughening of the high-manganese steel low in carbon embodied in my invention 105 can be carried out in a manner similar to that in which manganese steel as heretofore produced has been toughened. Examples of suitable toughening methods are described in former Letters Patent granted to me, to wit: 110 United States Patents Nos. 572891 and 731450.

If desired the manganese steel manufactured in accordance with my invention may contain other elements than iron, manganese and carbon, as for example, it may contain 5 nickel, chromium, tungsten, molybdenum and vanadium in varying proportions, say from one-tenth of one percent to thirty percent (.1% to 30%).

Having fully described my invention, what 10 I claim as new and desire to secure by Letters Patent is:—

1. The herein-described steel containing less than 1.0% of carbon and from 10% to 14% of manganese, capable of being readily 15 heat-treated and toughened in the mass with-

out cracking, and distinguished by its relatively strong magnetic character.

2. The herein-described steel containing less than 1.0% of carbon and a high percentage of manganese, distinguished by its relatively strong magnetic character, and capable of being readily heat-treated and toughened in the mass without cracking. 20

In testimony whereof, I have signed my name to this specification, in the presence of 25 two subscribing witnesses.

ROBERT ABBOTT HADFIELD.

Witnesses:

PERCY PHILLIPS,

ALFRED NUTTING.